

## UNITED STATES PATENT OFFICE

2,059,732

NITRIDED ALLOY STEEL COLD-DRAWING  
DIE

William Herbert Hatfield, Hathersage, England,  
assignor to Thos. Firth & John Brown Limited,  
Sheffield, England, a British company

No Drawing. Application July 24, 1934, Serial  
No. 736,785. In Great Britain July 25, 1933

5 Claims. (Cl. 148—31)

This invention comprises improvements in or relating to alloy steels, particularly for cold-drawing dies.

It is well known that for dies used in cold-drawing operations for the production of wire, tubes, and special sections of metals and alloys, a hard surface resistant to wear is necessary, since the hardness and resistance to wear affect the life of the die, the uniformity of dimensions and properties of the cold-drawn articles, and the amount of frictional resistance to passage through the die.

Alloy steels which have been surface-hardened by the so-called nitrogenizing process have already been used for cold-drawing dies. In the nitrogenizing process the alloy steel is subjected to the action of gases containing nitrogen in combined form (e.g. ammonia gas) at a temperature in the region of 500° C. The hardness of the core material of those alloys after nitrogenizing, which is practically the same as the general hardness of the alloy before nitrogenizing, is limited by the nature of the steel and by the fact that the prior treatment is such that a stable condition of the core material is reached which is unaffected subsequently by the temperature employed in the nitrogenizing operation. This prior treatment usually consists either of normalizing or hardening and tempering, and the hardness of the material when ready for the surface-hardening treatment usually lies between about 140 and 350 on the Brinell scale. The surface hardness after nitrogenizing may be as high as 1100 to 1150 on the diamond hardness scale.

In practice cold-drawing dies made from nitrogenized alloy steels have, in certain cases, been too weak to stand up to the heavy pressures involved in the drawing operations, owing to the fact that the thin nitrogenized skin has transmitted the pressure to the softer and more readily deformable core. The principal object of this invention is to provide an improved cold-drawing die which does not suffer from the above defect, and which at the same time provides a hard wear-resisting surface. This object is achieved by fabricating the die from an alloy steel of such a constitution that it is capable of surface-hardening by nitrogenizing and at the same time provides a body portion or core which may be, and shall remain after completion of the nitrogenizing process, sufficiently hard to be for all practical purposes undeformable.

According to the invention cold-drawing dies are made from a nitrogenized alloy steel having the normal composition of a high-speed tool steel

containing 8 to 25% tungsten, an effective amount up to 1% carbon, an effective amount up to 8% chromium, an effective amount up to 3% vanadium and, if desired, an effective amount up to 20% cobalt and/or an effective amount up to 8% molybdenum and normal proportions of other elements such as silicon and manganese, and modified by the further addition of an effective amount up to 2% aluminium. By the use of such an alloy a core hardness of the order of 550 Brinell or over can readily be obtained. While the invention is particularly concerned with the fabrication of cold-drawing dies, it includes alloy steels (for whatever purpose they may be subsequently used) which have the particular composition set out above and which have been subjected to the nitrogenizing process.

It is known that many high-speed tool steels are capable of a limited degree of surface-hardening by nitrogenizing but, according to the present invention, such surface-hardening is rendered more intense or of more practical service by the incorporation of aluminium, in the proportions defined above, in the steel.

It is to be noted that the present invention is concerned solely with the manufacture and use of a nitrogenized high-speed tool steel embodying as an essential constituent up to 2.0% aluminium. The application of the nitrogenizing process to alloy steels of other types which may contain aluminium has already been described. For example, British specification No. 174,580 describes the nitrogenizing of steel alloys containing aluminium, chromium, manganese, or silicon either separately or in any desired combination. Again in British specification No. 243,613 it is stated that articles which have their surface layers hardened by nitrogenization may assume—owing to the heating required for carrying out the operation of nitrogenization and the subsequent gradual cooling—a temper-brittle condition of the unhardened core-zone, and this condition can be remedied by using steel alloys which contain 0.5 to 2% of aluminium and, either separately or in any desired combination, silicon, manganese, nickel, chromium, molybdenum, tungsten, vanadium, titanium or zirconium amounting in all to from 0.5 to 4% and up to 0.6% of carbon. It has also been proposed to apply the process of nitrogenizing at a temperature of 550 to 950° C. to alloy steels of austenitic structure, and in some examples embodying that proposal the austenitic alloys contained up to 7% of aluminium. It is to be observed that none of these proposals is concerned with the nitrogenizing of an

alloy steel having the composition of a high-speed tool steel, nor with the use of such steels in cold-drawing dies.

In carrying out the present invention the tool steels, prior to nitrogenizing, may conveniently be treated by quenching or quickly cooling in oil, air or water from a high temperature, e. g. 1150° C., and tempering at a temperature not below 550° C., giving the well-known "red hard" condition. If desired, the tempering may be omitted as a separate process since the subsequent nitrogenizing process at a temperature in the region of 500° C. will, to a large degree, accomplish the tempering of the core material 15 without undue softening and, at the same time, produce a superhard skin.

A specific steel within this invention, on analysis showed the following composition:—

|           | Percent |
|-----------|---------|
| 20 Carbon | 0.39    |
| Silicon   | 0.22    |
| Manganese | 0.24    |
| Chromium  | 3.13    |
| 25 Nickel | 0.12    |
| Tungsten  | 10.27   |
| Vanadium  | 0.54    |
| Aluminium | 1.21    |

This steel, after being nitrogenized at a temperature of 500° C. for a period of four days, gave 30 the following hardness values using a Vickers' diamond hardness machine with a 30 kilogram load:—

|    | Depth be-<br>low surface<br>in mms. | Hardness        |  |
|----|-------------------------------------|-----------------|--|
|    |                                     | V. D. H.<br>No. |  |
| 35 | 0.10                                | 1325            |  |
|    | 0.20                                | 1325            |  |
| 40 | 0.29                                | 1099            |  |
|    | 0.38                                | 1024            |  |
|    | 0.48                                | 873             |  |
|    | 0.57                                | 527             |  |
|    | 0.76                                | 496             |  |
|    | 0.95                                | 476             |  |
| 45 | 1.14                                | 468             |  |
|    | 1.34                                | 470             |  |

In order to obtain the required hardness of the core, prior to nitrogenizing, the steel was oil quenched from 1150° C. and tempered at 580° C. 50 for one hour. It is noteworthy that the hardness of the core remains unchanged by the nitrogenizing treatment.

I claim:—

1. A cold-drawing die made from a nitrogenized alloy steel containing 8 to 25% of tungsten, an effective amount up to 1% of carbon, an effective amount up to 8% of chromium, an effective amount up to 3% of vanadium, an effective amount up to 20% of cobalt, and modified by the further addition of an effective amount to 5% amount to 2% of aluminium, the balance being iron together with such other alloying elements and impurities as are usual in alloy steels, the die being characterized by having a core-hardness of the order of 550 Brinell and a surface-hardness of upwards of 1100 on the diamond hardness scale.

2. A cold-drawing die made from a nitrogenized alloy steel containing 8 to 25% of tungsten, an effective amount up to 1% of carbon, an effective amount up to 8% of chromium, an effective amount up to 3% of vanadium, an effective amount up to 20% of cobalt, an effective amount up to 8% of molybdenum, and modified by the further addition of an effective amount to 20% amount to 2% of aluminium, the balance being iron together with such other alloying elements and impurities as are usual in alloy steels, the die being characterized by having a core-hardness of the order of 550 Brinell and a surface-hardness of upwards of 1100 on the diamond hardness scale.

3. A cold-drawing die having the core portion of a nitridable steel alloy containing tungsten from about 8 to about 25%, carbon from about 0.2 to about 1%, chromium from about 2 to about 8%, vanadium in an effective amount up to 3%, aluminium from about 0.2 to about 2%, and the remainder principally iron, said die having a core-hardness of the order of 550 Brinell even after being subjected to a temperature of about 500° C. and the working part having a surface-hardened by nitriding of the order of 1100 Brinell.

4. A process of surface hardening a cold drawing die which comprises nitriding a cold drawing die of high speed tool steel containing 8 to 25% of tungsten, an effective amount up to 1% of carbon, an effective amount up to 8% of chromium, an effective amount up to 3% of vanadium, an effective amount up to 2% of aluminium, the balance being iron together with such other alloying elements and impurities as are usually found in alloy steels; and treating the said steel prior to the nitriding by quenching from a temperature of the order of 1150° C.

5. The process set forth in claim 4, in which the steel is tempered at a temperature of the order of 550° C. after the step of quenching from 1150° C.

WILLIAM HERBERT HATFIELD.